

# UNITED STATES PATENT OFFICE.

GEORGE FRANKLIN ALLEN, OF GRANITE CITY, ILLINOIS, ASSIGNOR TO EDWARD R. HOYT,  
OF ST. LOUIS, MISSOURI.

## METALLIC PRODUCT.

No. 897,953.

Specification of Letters Patent.

Patented Sept. 8, 1908.

Application filed May 1, 1908. Serial No 430,265.

*To all whom it may concern:*

Be it known that I, GEORGE F. ALLEN, a citizen of the United States of America, residing in Granite City, county of Madison, and State of Illinois, have invented certain new and useful Improvements in Metallic Products, of which the following is a full, clear, and exact description.

My invention relates to a metallic product, 10 and it has for its object to produce a metallic product in which lead is contained as the major element and with which is combined another metal that will increase the tensile strength of the product.

15 My metallic product consists of two metals, lead and zinc, combined in such proportions that the zinc will greatly increase the tensile strength of the product, as compared with a metallic product in which only a

small percentage of zinc is combined with 20 lead. In making the product, I use zinc in the proportion of from three-fourths of one percent. to five percent., the balance of the product being lead, and preferably soft lead.

The metallic product herein described is of 25 particular utility in soft metal pipes, but may be used in the production of various other articles.

I claim:

A metal product consisting of from one 30 and four tenths percent. to five percent. of zinc and the balance of lead, substantially as set forth.

GEORGE FRANKLIN ALLEN.

In presence of—

E. S. KNIGHT,  
H. G. COOK.